

Aug. 6, 1974

HIROSHI TAKECHI ET AL

3,827,924

HIGH-STRENGTH ROLLED STEEL SHEETS

Filed May 19, 1972

3 Sheets-Sheet 1

FIG.1



FIG.2



Aug. 6, 1974

HIROSHI TAKECHI ET AL

3,827,924

HIGH-STRENGTH ROLLED STEEL SHEETS

Filed May 19, 1972

FIG.3

3 Sheets-Sheet 2



FIG.4



Aug. 6, 1974

HIROSHI TAKECHI ET AL

3,827,924

HIGH-STRENGTH ROLLED STEEL SHEETS

Filed May 19, 1972

3 Sheets-Sheet 3

FIG.5



FIG.6



3,827,924

**HIGH-STRENGTH ROLLED STEEL SHEETS**  
 Hiroshi Takechi, Kisarazu, and Hiroaki Masui, Minoru  
 Kawaharada, and Motoaki Sugiyama, Kitakyushu,  
 Japan, assignors to Nippon Steel Corporation, Tokyo,  
 Japan

Filed May 19, 1972, Ser. No. 255,019

Claims priority, application Japan, May 21, 1971,  
 46/34,625; Feb. 12, 1972, 47/14,321

Int. Cl. C22c 29/00

U.S. Cl. 148—36

2 Claims

## ABSTRACT OF THE DISCLOSURE

A high-strength rolled steel sheet of chemical composition comprising;

C: 0.02—0.10%, Si $\leq$ 0.7%, Mn: 0.01—0.70%,  
 P: 0.05—0.25%, Al: 0.005—0.100%

with the balance being iron and unavoidable impurities.

The present invention relates to a high-strength rolled steel sheet having good drawability, impact-resistance, corrosion-resistance and coatability.

The term "rolled steel sheet" used in the present invention should be understood to include hot rolled steel sheets and cold rolled steel sheets obtained from the hot rolled steel sheets by cold rolling, recrystallization annealing and skin-pass rolling.

Recently, high-strength cold rolled steel sheets have been used increasingly in many parts of the outer skins and inner skins of automobiles for safety purposes. Such high-strength cold rolled steel sheets suitable for such applications must have various properties to withstand for severe service conditions, and among them the following properties are required.

1. Excellent drawability as well as high-strength as compared with that of ordinary cold rolled steel sheets for general use, and little susceptibility to embrittlement.
2. Excellent corrosion-resistance and coatability as automobile trims.

Among the factors indicating elongation and ductility of steel sheets, the workhardening index  $n$  is used. This  $n$  value is a value given by the ratio of the tensile strength  $\delta$  (or yield point) and strain  $\epsilon$ , namely

$$n = \frac{d \log \delta}{d \log \epsilon}$$

A large  $n$  value shows better elongation and ductility of the steel sheet, and this value lowers as the tensile strength of the steel sheet increases.

Further, steel sheets have the tendency of secondary work cracking under which embrittlement or pseudo-embrittlement destruction occurs is due to loads imposed on work-pieces by deep-drawing. In general, the secondary work test is done to determine if destruction (or cracking) is results on the side wall portion etc. of a cup test sample by drawing a steel sheet having an 80—160 mm. diameter with an appropriate ratio of reduction area (ratio of primary drawing). The thus obtained cup test sample is given loads continuously up to a maximum load of 3000 ton in a vessel containing ice and water. Generally, the larger limit ratio of primary drawing which does not cause cracking indicates a better secondary workability.

Meanwhile, the drawability of cold rolled steel sheets may be determined by the  $\bar{r}$  value which is the average plastic strain ratio of a plastic strain ratio ( $\bar{r}$  value) expressed by the ratio of sheet width strain and sheet thick-

ness strain, and thus the drawability may be expressed by the following formula

$$\bar{r} = (r_0 + 2r_{45} + r_{90}) \div 4$$

$r_0$  =  $r$  value in the rolling direction

5  $r_{45}$  =  $r$  value in a direction at 45° to the rolling direction

$r_{90}$  =  $r$  value in a direction at 90° to the rolling direction.

10 In general, a large  $\bar{r}$  value indicates better drawability, and ordinary Al-killed steels show an  $\bar{r}$  value of about 1.6, and rimmed steels show an  $\bar{r}$  value of about 1.3.

In the case of cold rolled steel sheets, many experiments and studies have been made with respect to the addition of special elements and thermal production methods chiefly for the purpose of improving drawability alone instead of improving both strength and drawability. However, even with a cold rolled steel sheet having both high strength and high  $\bar{r}$  value, its application would be limited

15 unless the products obtained by drawing are not susceptible to embrittlement cracking. The embrittlement cracking usually takes place in drawn products having a larger ratio of reduction of area, and as for the method for determining the cracking tendency, the secondary work test as mentioned above is adopted.

20 Further, in the case of cold rolled steel sheets, better surface properties, such as, rust-proofness and coatability as required by automobile applications and house surfacing materials and building construction surface materials have been increasingly in demand.

25 Therefore, the object of the present invention is to provide a high-strength cold rolled steel sheet which overcomes the above defects and satisfies the above demands and the present invention is based on the discovery that high P content, Si-P cold rolled steel sheets containing B, Al and Si or containing lowered oxygen content shows excellent material qualities and surface properties.

The basic composition of the present inventive steel is:

30 C: 0.02—0.10%, Si $\leq$ 0.7, Mn: 0.01—0.70%,  
 P: 0.05—0.25%, Al: 0.005—0.10%

35 with the balance being iron and unavoidable impurities and this basic composition is modified by the addition of 0.002—0.01% of boron or by reducing the oxygen content to 0.015% or less.

40 Typical embodiments of the present inventive steel comprises:

45 C: 0.02—0.10%, Si $\leq$ 0.7%, Mn: 0.01—0.60%,  
 P: 0.05—0.25%, Al: 0.005—0.100%,  
 B: 0.002—0.010%

50 with the balance being iron and unavoidable impurities, or

55 C: 0.025—0.100%, Si: 0.11—0.69%,  
 Mn: 0.01—0.70%, P: 0.06—0.16%  
 sol. Al: 0.01—0.10%, oxygen $\leq$ 0.015%

60 with the balance being iron and unavoidable impurities.

65 Reasons for the limitation of each element in the present invention are as follows:

Carbon is an element effective for increasing the strength of steel sheets, but it is rather used as an element for improving impact secondary workability. Less than 0.02% of carbon is not effective, while excessive carbon content forms large cementite and lowers the ductility impact secondary workability and the  $\bar{r}$  value. Therefore, the upper limit of the carbon content is set at 0.100%.

70 Silicon is effective for increasing strength, but in the present invention it contributes to prevent the lowering of the impact secondary workability due to phosphorus and more than 0.11% of Si is required.

But silicon contents of more than 0.69% tend to deteriorate the improved rust-proofness and coatability contributed by the phosphorus content.

Manganese is effective for increasing the strength and is contained as an important component for high tensile strength steel sheets. In the present invention, more than 0.01% of Mn is required for increasing the strength and preventing hot embrittlement during hot rolling. But manganese contents of more than 0.70% will lower the drawability and rust-proofness improved by phosphorus content.

More than 0.05% of phosphorus is required for improving the strength, drawability as well as the coatability and rust-proofness, but more than 0.16% of phosphorus will deteriorate the impact secondary workability. Boron is added to prevent the deterioration of impact secondary workability caused by addition of phosphorus more than 0.16% and thus phosphorus can be safely added to up to 0.25%, but a preferred range of phosphorus content is 0.08–0.15%. More than about 0.002% of boron is necessary for the above purpose but excessive boron content will deteriorate ductility, press formability and cause surface cracking of hot rolled slabs. Thus, the boron content is limited to 0.002–0.010%.

In general, aluminum acts as a deoxidizing agent and the present inventors have found that aluminum is effective for preventing deterioration of the impact secondary workability, and at least 0.01% of aluminum in the form of soluble aluminum is required for the above purpose in the case where no boron is added. On the other hand, when boron is added, aluminum is an amount more than 0.005% enhances the effect of boron by being combined with oxygen and nitrogen in the metal to improve the secondary workability. But an excessive aluminum content increases the alumina content to deteriorate the surface properties with only little improvement in its desirable effect. Thus the upper limit of aluminium is limited to 0.10% in the form of soluble aluminum.

Silicon is an effective element for deoxidation and improvement of strength, and is necessary in the present invention for improvement of the secondary workability thus increasing the effect of boron addition by combination with oxygen just as aluminium. But more than 0.7% of silicon will lower ductility and should be avoided because it damages the press formability.

Oxygen is present in the steel as non-metallic inclusions and in a solid solution state in a very small amount. When oxygen is present in an amount of more than 0.015%, it has been found, that impact secondary workability is remarkably deteriorated and oxidizes useful elements, such as, silicon and phosphorus and lower their effectiveness. Therefore, the upper limit of the oxygen content is set at 0.015% and the oxygen content should be as low as possible.

Unavoidable impurities, such as, sulfur which bars the object of the present invention and often causes crackings during the production of cold rolled steel sheets, should be kept as low as possible.

The high strength cold rolled steel sheets of the present invention are produced by making steel of the above composition in a converter or an electric furnace, making ingots from the steel, breaking the ingots into slabs, or continuous-casting the steel into slabs, hot rolling the slabs, acid pickling and cold rolling the hot rolled plates with a reduction rate of more than 30%, box annealing or continuously annealing the sheets at a temperature between 550° C.–900° C., and then skin-pass rolling the sheets with a reduction rate between 0.2–3.0%.

The present invention will be better understood from the following examples.

#### Example 1

Steel having a chemical composition shown in Table 1 was prepared in a 1-ton electric furnace. Thus obtained

steel ingot was soaked for one hour at 1250° C., hot rolled at 900° C. at a finishing temperature of 900° C. to obtain a hot rolled plate of 2.7 mm. thickness, and the hot rolled plate was cold rolled at a reduction rate of 70%, subjected to a batch type recrystallization annealing in which the sheet was kept at 710° C. for 4 hours and then furnace cooled, and then skin-pass rolling at a reduction rate of 1.2% to obtain cold rolled steel sheets. JIS No. 5 tensile test samples were prepared from the above obtained cold rolled sheets and subjected to an ordinary tensile test by a tensile test machine of instron type to determine yield point, tensile and  $n$  values. The test results are shown in Table 1. The  $n$  value was obtained by the following formula;

15

$$n = (n_0 + 2n_{45} + n_{90}) \div 4$$

20

in which  $n_0 = n$  value in the rolling direction of the sheet  
 $n_{45} = n$  value in a direction at 45° to the rolling direction  
 $n_{90} = n$  value in a direction at 90° to the rolling direction.

25

The yield point and tensile strength values were obtained by the same method.

#### Example 2

Table 3 shows chemical compositions of cold rolled steel sheets of 0.8 mm. thickness produced by making ingots from molten steel prepared in a convertor, breaking down the ingots and hot rolling the slabs into hot rolled steel plates of 2.7 mm. thickness and cold rolling the hot rolled plates.

35

The cold rolled steel sheets were further subjected to recrystallization annealing at 710° C. for 4 hours, and to skin-pass rolling at a reduction rate of 1.2% to obtain the high-strength cold rolled steel sheets (A–H) of the present invention. The steel sheets (I–X) are shown in Table 3 for comparison.

40

Tensile strength values of these steel sheets are shown in Table 3 and  $n$  values are shown in FIG. 3 and the limit drawing ratio values obtained by the impact secondary working test (these values were obtained for samples prepared by making the outer circumference of steel blanks before primary drawing) are shown in FIG. 4, rust-proofness and coatability are shown in FIG. 5 and FIG. 6, respectively. The coatability was determined by paint adhesion test. The paint adhesion test is done by subjecting the steel sheet to phosphate treatment and determining the diameter phosphate crystal grains and the number of phosphate nuclei per unit area (1 cm.<sup>2</sup>) of the sheet. A smaller diameter of phosphate crystal grains, and a larger number of phosphate nuclei indicate better coatability.

45

The present steel sheets show better properties than those of the comparative steel sheets, and particularly in respect of the results of the paint adhesion test shown in FIG. 6, the present inventive steel sheets show a phosphate crystal grain diameter of about 11–15 $\mu$  and phosphate nuclei of about 130–170 $\times 10^4$ /cm.<sup>2</sup> as compared with a phosphate crystal grain diameter of about 15–17 $\mu$  and phosphate nuclei of about 70–90 $\times 10^4$ /cm.<sup>2</sup> of ordinary rimmed soft steels, thus indicating the excellent coatability of the present inventive steel sheets.

50

It should be noted in this point that the present inventive steel sheet shows an excellent value in respect of each of drawability, impact secondary workability rust-proofness and coatability (paint adhesion) as shown in FIG. 3 to FIG. 6. In case of the comparative steel sheets, one or more of these properties are remarkably poor and thus very unsatisfactory for the applications aimed by the present invention, and are greatly limited their use as high-strength cold rolled steel sheet.

75

TABLE 1  
(Samples A8-A10, A14-A17: Inventive steel sheets, Samples A1-A9,  
A11-A13, A18, B1-B12: Comparative steel sheets)

| Samples | Chemical compositions (weight percent) |       |      |       |       |       |       |        |       |
|---------|----------------------------------------|-------|------|-------|-------|-------|-------|--------|-------|
|         | C                                      | P     | Mn   | S     | Si    | O     | Al    | B      | N     |
| A1..... | 0.054                                  | 0.07  | 0.31 | 0.018 | 0.018 | 0.042 | 0.002 | <0.001 | 0.004 |
| A2..... | 0.048                                  | 0.15  | 0.26 | 0.022 | 0.016 | 0.038 | 0.004 | <0.001 | 0.003 |
| A3..... | 0.068                                  | 0.19  | 0.28 | 0.016 | 0.024 | 0.036 | 0.002 | <0.001 | 0.004 |
| A4..... | 0.051                                  | 0.18  | 0.30 | 0.024 | 0.224 | 0.009 | 0.004 | <0.001 | 0.004 |
| A5..... | 0.065                                  | 0.17  | 0.27 | 0.014 | 0.035 | 0.006 | 0.038 | <0.001 | 0.006 |
| A6..... | 0.046                                  | 0.15  | 0.25 | 0.015 | 0.286 | 0.003 | 0.033 | <0.001 | 0.007 |
| A7..... | 0.054                                  | 0.14  | 0.32 | 0.022 | 0.018 | 0.034 | 0.003 | 0.005  | 0.004 |
| A8..... | 0.046                                  | 0.15  | 0.29 | 0.023 | 0.021 | 0.016 | 0.012 | 0.004  | 0.005 |
| A9..... | 0.043                                  | 0.16  | 0.26 | 0.026 | 0.018 | 0.004 | 0.072 | 0.002  | 0.008 |
| A10.... | 0.029                                  | 0.18  | 0.28 | 0.024 | 0.028 | 0.002 | 0.042 | 0.008  | 0.007 |
| A11.... | 0.054                                  | 0.16  | 0.34 | 0.018 | 0.183 | 0.006 | 0.002 | 0.008  | 0.003 |
| A12.... | 0.044                                  | 0.17  | 0.22 | 0.015 | 0.165 | 0.007 | 0.004 | 0.007  | 0.004 |
| A13.... | 0.026                                  | 0.16  | 0.34 | 0.024 | 0.320 | 0.008 | 0.004 | 0.005  | 0.004 |
| A14.... | 0.048                                  | 0.17  | 0.31 | 0.016 | 0.494 | 0.002 | 0.038 | 0.007  | 0.006 |
| A15.... | 0.062                                  | 0.15  | 0.25 | 0.019 | 0.263 | 0.003 | 0.065 | 0.002  | 0.007 |
| A16.... | 0.035                                  | 0.15  | 0.29 | 0.026 | 0.286 | 0.005 | 0.011 | 0.005  | 0.004 |
| A17.... | 0.029                                  | 0.21  | 0.28 | 0.018 | 0.126 | 0.003 | 0.034 | 0.009  | 0.006 |
| A18.... | 0.073                                  | 0.08  | 0.33 | 0.016 | 0.114 | 0.008 | 0.003 | <0.001 | 0.000 |
| B1..... | 0.046                                  | <0.01 | 0.72 | 0.022 | 0.013 | 0.042 | 0.002 | <0.001 | 0.003 |
| B2..... | 0.038                                  | <0.01 | 1.54 | 0.018 | 0.024 | 0.028 | 0.004 | <0.001 | 0.004 |
| B3..... | 0.054                                  | <0.01 | 2.63 | 0.019 | 0.026 | 0.033 | 0.006 | <0.001 | 0.004 |
| B4..... | 0.046                                  | <0.01 | 0.36 | 0.024 | 0.524 | 0.006 | 0.003 | <0.001 | 0.003 |
| B5..... | 0.051                                  | <0.01 | 0.29 | 0.016 | 0.918 | 0.006 | 0.002 | <0.001 | 0.003 |
| B6..... | 0.049                                  | <0.01 | 0.34 | 0.018 | 1.382 | 0.005 | 0.004 | <0.001 | 0.003 |
| B7..... | 0.031                                  | <0.01 | 0.31 | 0.014 | 0.018 | 0.002 | 0.843 | <0.001 | 0.007 |
| B8..... | 0.058                                  | <0.01 | 0.28 | 0.023 | 0.021 | 0.003 | 1.241 | <0.001 | 0.009 |
| B9..... | 0.064                                  | <0.01 | 0.26 | 0.009 | 0.019 | 0.002 | 1.935 | <0.001 | 0.009 |
| B10.... | 0.124                                  | <0.01 | 0.24 | 0.018 | 0.026 | 0.044 | 0.005 | <0.001 | 0.004 |
| B11.... | 0.116                                  | <0.01 | 0.52 | 0.016 | 0.014 | 0.031 | 0.004 | <0.001 | 0.004 |
| B12.... | 0.129                                  | <0.01 | 0.86 | 0.023 | 0.018 | 0.024 | 0.004 | <0.001 | 0.003 |

| Samples | Mechanical properties                  |                                             |         |  |  |  |  |  |  |
|---------|----------------------------------------|---------------------------------------------|---------|--|--|--|--|--|--|
|         | Yield point<br>(kg./mm. <sup>2</sup> ) | Tensile strength<br>(kg./mm. <sup>2</sup> ) | n Value |  |  |  |  |  |  |
| A1..... | 32.1                                   | 40.4                                        | 0.237   |  |  |  |  |  |  |
|         | 27.2                                   | 39.3                                        | 0.246   |  |  |  |  |  |  |
| A2..... | 34.1                                   | 43.3                                        | 0.238   |  |  |  |  |  |  |
|         | 29.6                                   | 41.8                                        | 0.254   |  |  |  |  |  |  |
| A3..... | 37.8                                   | 47.3                                        | 0.239   |  |  |  |  |  |  |
|         | 33.4                                   | 46.2                                        | 0.248   |  |  |  |  |  |  |
| A4..... | 40.1                                   | 49.2                                        | 0.212   |  |  |  |  |  |  |
|         | 35.6                                   | 48.6                                        | 0.217   |  |  |  |  |  |  |
| A5..... | 36.9                                   | 44.6                                        | 0.232   |  |  |  |  |  |  |
|         | 32.1                                   | 43.9                                        | 0.247   |  |  |  |  |  |  |
| A6..... | 35.1                                   | 45.2                                        | 0.229   |  |  |  |  |  |  |
|         | 31.2                                   | 43.2                                        | 0.236   |  |  |  |  |  |  |
| A7..... | 32.9                                   | 41.2                                        | 0.246   |  |  |  |  |  |  |
|         | 28.8                                   | 40.6                                        | 0.258   |  |  |  |  |  |  |
| A8..... | 35.4                                   | 42.3                                        | 0.260   |  |  |  |  |  |  |
|         | 29.7                                   | 41.5                                        | 0.267   |  |  |  |  |  |  |
| A9..... | 36.1                                   | 43.1                                        | 0.252   |  |  |  |  |  |  |
|         | 30.4                                   | 42.4                                        | 0.261   |  |  |  |  |  |  |
| A10.... | 37.1                                   | 46.1                                        | 0.231   |  |  |  |  |  |  |
|         | 32.2                                   | 45.1                                        | 0.246   |  |  |  |  |  |  |
| A11.... | 35.2                                   | 44.5                                        | 0.223   |  |  |  |  |  |  |
|         | 31.6                                   | 43.7                                        | 0.240   |  |  |  |  |  |  |
| A12.... | 39.4                                   | 48.8                                        | 0.203   |  |  |  |  |  |  |
|         | 35.6                                   | 47.4                                        | 0.219   |  |  |  |  |  |  |
| A13.... | 35.1                                   | 45.6                                        | 0.225   |  |  |  |  |  |  |
|         | 31.9                                   | 44.1                                        | 0.233   |  |  |  |  |  |  |
| A14.... | 39.6                                   | 47.2                                        | 0.219   |  |  |  |  |  |  |
|         | 34.8                                   | 46.5                                        | 0.227   |  |  |  |  |  |  |
| A15.... | 35.1                                   | 43.4                                        | 0.232   |  |  |  |  |  |  |
|         | 31.5                                   | 42.2                                        | 0.248   |  |  |  |  |  |  |
| A16.... | 35.2                                   | 43.6                                        | 0.258   |  |  |  |  |  |  |
|         | 31.3                                   | 42.8                                        | 0.271   |  |  |  |  |  |  |
| A17.... | 40.7                                   | 49.8                                        | 0.208   |  |  |  |  |  |  |
|         | 35.9                                   | 48.7                                        | 0.210   |  |  |  |  |  |  |
| A18.... | 32.8                                   | 41.0                                        | 0.219   |  |  |  |  |  |  |
|         | 28.4                                   | 40.1                                        | 0.238   |  |  |  |  |  |  |
| B1..... | 26.1                                   | 31.9                                        | 0.263   |  |  |  |  |  |  |
|         | 21.4                                   | 31.2                                        | 0.267   |  |  |  |  |  |  |
| B2..... | 29.2                                   | 36.3                                        | 0.236   |  |  |  |  |  |  |
|         | 24.8                                   | 35.1                                        | 0.242   |  |  |  |  |  |  |
| B3..... | 36.6                                   | 44.2                                        | 0.201   |  |  |  |  |  |  |
|         | 32.1                                   | 43.6                                        | 0.208   |  |  |  |  |  |  |
| B4..... | 30.4                                   | 37.7                                        | 0.224   |  |  |  |  |  |  |
|         | 25.3                                   | 36.1                                        | 0.238   |  |  |  |  |  |  |

TABLE 1—Continued  
Mechanical properties

| Samples | Yield point<br>(kg./mm. <sup>2</sup> ) | Tensile strength<br>(kg./mm. <sup>2</sup> ) | n Value |   |    |    |    |    |    |
|---------|----------------------------------------|---------------------------------------------|---------|---|----|----|----|----|----|
|         |                                        |                                             |         | 5 | 10 | 15 | 20 | 25 | 30 |
| B5..... | 34.8                                   | 43.6                                        | 0.196   |   |    |    |    |    |    |
|         | 30.6                                   | 42.4                                        | 0.207   |   |    |    |    |    |    |
| B6..... | 38.2                                   | 47.1                                        | 0.192   |   |    |    |    |    |    |
|         | 34.8                                   | 46.2                                        | 0.201   |   |    |    |    |    |    |
| B7..... | 29.4                                   | 36.1                                        | 0.238   |   |    |    |    |    |    |
|         | 24.9                                   | 35.6                                        | 0.247   |   |    |    |    |    |    |
| B8..... | 32.6                                   | 38.0                                        | 0.242   |   |    |    |    |    |    |
|         | 28.0                                   | 37.9                                        | 0.246   |   |    |    |    |    |    |
| B9..... | 34.1                                   | 43.1                                        | 0.215   |   |    |    |    |    |    |
|         | 30.9                                   | 42.3                                        | 0.224   |   |    |    |    |    |    |
| B10.... | 28.4                                   | 37.8                                        | 0.214   |   |    |    |    |    |    |
|         | 24.9                                   | 36.2                                        | 0.228   |   |    |    |    |    |    |
| B11.... | 31.8                                   | 39.2                                        | 0.193   |   |    |    |    |    |    |
|         | 27.1                                   | 38.7                                        | 0.205   |   |    |    |    |    |    |
| B12.... | 36.2                                   | 41.2                                        | 0.206   |   |    |    |    |    |    |
|         | 32.1                                   | 40.8                                        | 0.217   |   |    |    |    |    |    |

TABLE 2

25 (Samples A8-A10, A14-A17: Inventive steel sheets Samples A1-A4, A7-A9, A11-A13, A18: Comparative steel sheets)

| Samples | Chemical Compositions (weight percent) |      |      |       |       |       |       |       |       |
|---------|----------------------------------------|------|------|-------|-------|-------|-------|-------|-------|
|         | C                                      | P    | Mn   | S     | Si    | O     | Al    | B     | N     |
| A1..... | 0.054                                  | 0.07 | 0.31 | 0.018 | 0.018 | 0.042 | 0.002 | ..... | 0.00  |
| A2..... | 0.048                                  | 0.15 | 0.26 | 0.022 | 0.016 | 0.038 | 0.004 | ..... | 0.004 |
| A3..... | 0.068                                  | 0.19 | 0.28 | 0.016 | 0.024 | 0.036 | 0.002 | ..... | 0.003 |
| A4..... | 0.051                                  | 0.18 | 0.30 | 0.024 | 0.224 | 0.009 | 0.004 | ..... | 0.004 |
| A7....  | 0.054                                  | 0.14 | 0.32 | 0.022 | 0.018 | 0.034 | 0.003 | 0.008 | 0.004 |
| A8....  | 0.046                                  | 0.15 | 0.29 | 0.023 | 0.021 | 0.016 | 0.012 | 0.004 | 0.004 |
| A9....  | 0.043                                  | 0.16 | 0.26 | 0.026 | 0.018 | 0.004 | 0.072 | 0.002 | 0.008 |
| A10.... | 0.029                                  | 0.18 | 0.28 | 0.024 | 0.028 | 0.002 | 0.042 | 0.008 | 0.007 |
| A11.... | 0.054                                  | 0.16 | 0.34 | 0.018 | 0.183 | 0.006 | 0.002 | 0.008 | 0.004 |
| A12.... | 0.044                                  | 0.17 | 0.22 | 0.015 | 0.616 | 0.007 | 0.004 | 0.007 | 0.003 |
| A13.... | 0.026                                  | 0.16 | 0.34 | 0.024 | 0.320 | 0.008 | 0.004 | 0.005 | 0.004 |
| A14.... | 0.048                                  | 0.17 | 0.31 | 0.016 | 0.494 | 0.002 | 0.038 | 0.007 | 0.006 |
| A15.... | 0.062                                  | 0.15 | 0.25 | 0.019 | 0.263 | 0.003 | 0.065 | 0.002 | 0.007 |
| A16.... | 0.035                                  | 0.15 | 0.29 | 0.026 | 0.286 | 0.005 | 0.011 | 0.005 | 0.004 |
| A17.... | 0.029                                  | 0.21 | 0.28 | 0.018 | 0.126 | 0.003 | 0.034 | 0.009 | 0.006 |
| A18.... | 0.073                                  | 0.08 | 0.33 | 0.016 | 0.114 | 0.008 | 0.003 | ..... | 0.003 |

Secondary workability

| Samples | Rate of primary reduction of area |     |     |     |     |     |
|---------|-----------------------------------|-----|-----|-----|-----|-----|
|         | 1.8                               | 2.2 | 2.6 | 3.0 | 3.4 | 3.8 |
| A1..... | O                                 | ●   | X   | ⊗   | X   | ⊗   |
| A2..... | O                                 | ⊗   | X   | ⊗   | X   | ⊗   |
| A3..... | O                                 | ⊗   | X   | ⊗   | X   | ⊗   |
| A4..... | O                                 | ⊗   | X   | ⊗   | X   |     |

TABLE 3

| Samples             | Chemical Compositions (weight percent) |      |       |      |       |            |       | Tensile strength<br>(kg./mm. <sup>2</sup> ) |
|---------------------|----------------------------------------|------|-------|------|-------|------------|-------|---------------------------------------------|
|                     | C                                      | Si   | P     | Mn   | S     | Sol.<br>Al | O     |                                             |
| Inventive steels:   |                                        |      |       |      |       |            |       |                                             |
| A                   | 0.046                                  | 0.18 | 0.144 | 0.28 | 0.012 | 0.024      | 0.007 | 48.2                                        |
| B                   | 0.029                                  | 0.52 | 0.096 | 0.14 | 0.018 | 0.013      | 0.011 | 46.4                                        |
| C                   | 0.076                                  | 0.31 | 0.074 | 0.34 | 0.016 | 0.042      | 0.006 | 42.8                                        |
| D                   | 0.032                                  | 0.61 | 0.113 | 0.52 | 0.012 | 0.027      | 0.010 | 48.0                                        |
| E                   | 0.086                                  | 0.25 | 0.108 | 0.61 | 0.011 | 0.034      | 0.005 | 45.9                                        |
| F                   | 0.057                                  | 0.33 | 0.136 | 0.08 | 0.018 | 0.032      | 0.009 | 47.7                                        |
| G                   | 0.092                                  | 0.14 | 0.088 | 0.24 | 0.009 | 0.062      | 0.005 | 43.4                                        |
| H                   | 0.061                                  | 0.42 | 0.151 | 0.37 | 0.010 | 0.016      | 0.011 | 50.6                                        |
| Comparative steels: |                                        |      |       |      |       |            |       |                                             |
| I                   | 0.016                                  | 0.26 | 0.122 | 0.26 | 0.012 | 0.024      | 0.009 | 47.0                                        |
| J                   | 0.021                                  | 0.41 | 0.086 | 0.29 | 0.007 | 0.042      | 0.008 | 45.1                                        |
| K                   | 0.113                                  | 0.15 | 0.103 | 0.19 | 0.014 | 0.020      | 0.010 | 44.6                                        |
| L                   | 0.043                                  | 0.09 | 0.125 | 0.22 | 0.012 | 0.041      | 0.008 | 44.9                                        |
| M                   | 0.031                                  | 0.81 | 0.104 | 0.28 | 0.013 | 0.036      | 0.007 | 48.6                                        |
| N                   | 0.036                                  | 0.97 | 0.087 | 0.32 | 0.014 | 0.039      | 0.008 | 48.1                                        |
| O                   | 0.028                                  | 0.27 | 0.046 | 0.26 | 0.009 | 0.031      | 0.007 | 38.4                                        |
| P                   | 0.051                                  | 0.22 | 0.007 | 0.31 | 0.011 | 0.028      | 0.003 | 34.2                                        |
| Q                   | 0.048                                  | 0.52 | 0.029 | 0.36 | 0.010 | 0.071      | 0.005 | 38.7                                        |
| R                   | 0.064                                  | 0.34 | 0.172 | 0.24 | 0.013 | 0.042      | 0.006 | 53.2                                        |
| S                   | 0.042                                  | 0.42 | 0.195 | 0.38 | 0.012 | 0.035      | 0.008 | 55.4                                        |
| T                   | 0.036                                  | 0.24 | 0.126 | 0.84 | 0.009 | 0.028      | 0.008 | 48.2                                        |
| U                   | 0.041                                  | 0.62 | 0.097 | 0.27 | 0.008 | 0.008      | 0.015 | 47.4                                        |
| V                   | 0.034                                  | 0.48 | 0.114 | 0.34 | 0.008 | 0.006      | 0.017 | 47.8                                        |
| W                   | 0.042                                  | 0.24 | 0.106 | 0.28 | 0.012 | 0.009      | 0.022 | 45.0                                        |
| X                   | 0.032                                  | 0.28 | 0.118 | 0.29 | 0.014 | 0.011      | 0.019 | 47.1                                        |

and having a yield point in the range from 29.7 to 35.9 kg./mm.<sup>2</sup> and an *n* value from 0.210 to 0.267.

2. A high-strength rolled steel sheet consisting essentially of

C: 0.025-0.100%, Si: 0.11-0.69%,  
Mn: 0.01-0.70%, P: 0.06-0.16%,

Al: 0.01-0.10%, and Oxygen  $\leq$  0.015%,

with the balance being iron and unavoidable impurities, and having a yield point in the range from 29.7 to 35.9 kg./mm.<sup>2</sup> and an *n* value from 0.210 to 0.267.

#### References Cited

##### UNITED STATES PATENTS

|           |         |                           |          |
|-----------|---------|---------------------------|----------|
| 3,239,390 | 3/1966  | Matsukura et al. _____    | 148-12   |
| 3,496,032 | 2/1970  | Shimizu (I) et al. _____  | 148-12   |
| 3,188,250 | 6/1965  | Holbein et al. _____      | 148-120  |
| 3,668,016 | 6/1972  | Shimizu (II) et al. _____ | 148-36   |
| 2,772,154 | 11/1956 | Morgan et al. _____       | 75-123 B |
| 3,347,718 | 10/1967 | Carpenter et al. _____    | 148-111  |
| 3,709,744 | 1/1973  | Goodman et al. _____      | 148-36   |
| 3,244,565 | 4/1966  | Mayer et al. _____        | 148-12.1 |
| 3,404,047 | 10/1968 | Goodman et al. _____      | 148-12.1 |
| 3,537,913 | 11/1970 | Klisowski _____           | 148-36   |

25 WALTER R. SATTERFIELD, Primary Examiner

U.S. Cl. X.R.

75-123 B; 148-12, 122

What is claimed is:

1. A high-strength rolled steel sheet consisting essentially

of

C: 0.02-0.10%; Si  $\leq$  0.7%, Mn: 0.01-0.60%,

P: 0.05-0.25%, Al: 0.005-0.10%,

B: 0.002-0.010%, and 0.005 to 0.008% N

with the balance being iron and unavoidable impurities,

30